

# UNITED STATES PATENT OFFICE.

JOHN C. BRADLEY, OF BUFFALO, NEW YORK.

## METHOD OF RENDERING IRON CASTINGS MALLEABLE.

SPECIFICATION forming part of Letters Patent No. 637,369, dated November 21, 1899.

Application filed August 14, 1899. Serial No. 727,236. (No specimens.)

*To all whom it may concern:*

Be it known that I, JOHN C. BRADLEY, a citizen of the United States, residing in Buffalo, county of Erie, and State of New York, 5 have invented a new and useful Improvement in Methods of Rendering Iron Castings Malleable, of which the following is a specification.

In the process of rendering iron castings 10 malleable as ordinarily practiced the iron castings are packed in annealing pots or boxes, together with steel scale, wrought-iron bittings or turnings, or other small particles of iron, which material has been treated with 15 sal-ammoniac or to which sal-ammoniac has been added. These pots or boxes are then placed in the annealing-kiln and exposed to a high degree of heat for a suitable period of time, as the nature of the castings may require. 20 In the cast-iron of which such castings are formed the carbon is combined with the iron, and such castings show a white fracture when broken, while in the annealed castings the percentage of carbon is less than in the original 25 state and the carbon which remains is uncombined or in the graphitic state, so that the annealed castings show a blackish or dark-blue fracture. The material which is used for this packing—such as steel scale, 30 wrought-iron scale, wrought-iron turnings—is expensive, and its treatment with sal-ammoniac increases the expense. Furthermore, this material fuses at a comparatively low temperature and often cakes at the annealing 35 heat to such an extent that it adheres tenaciously to the castings and pots, so that it always involves considerable labor to remove the castings from the pots and to free the annealed castings from the adhering packing 40 material, which is particularly difficult when the castings are intricate or have recesses, cavities, or crevices. The packing material often becomes so lumpy during the annealing process that it must be pulverized 45 before it can be used again.

The object of my invention is to overcome these difficulties and to reduce the cost of annealing such castings.

In practicing my invention I pack the iron 50 castings in furnace-slag which is rich in iron oxide and which has been coarsely pulverized

or reduced to a granular condition. Slag from a reverberatory, open-hearth, or other furnace in which iron or steel is melted is suitable for this purpose. Such slag usually 55 contains from thirty to fifty per cent. of iron oxide. This slag is crushed, coarsely pulverized, or granulated in any suitable manner, which can be readily done, because such slag is usually more or less friable. The castings 60 are packed in the pots with this pulverized, granulated, or crushed slag and are subjected to heat in the annealing-kiln in the usual manner. This packing material does not fuse or cake at the annealing heat and therefore 65 does not adhere to the annealed castings, but remains granular and leaves the castings and the pots readily, so that the castings are removed from the pots freely and in a clean condition, unencumbered by adhering pack- 70 ing material. This packing material reduces the percentage of the carbon in the castings very effectively and changes the remaining carbon to the graphitic state, producing an- 75 nealed or malleable-iron castings of excellent quality. This packing material is a waste product of the iron furnace and is of no value. It can be made ready for use at trifling cost, as it only requires to be crushed or pulverized, and as it does not fuse or cake it re- 80 mains in the proper condition for use. The use of this packing material avoids the heavy expense attending the use of the materials heretofore used for this purpose, which ex- 85 pense arises both from the cost of the mate- rial and the cost of cleaning the castings and retaining the material in the proper condi- tion for use.

I claim as my invention—

The herein-described method of annealing 90 iron castings which consists in packing the castings in pulverized furnace-slag which is rich in iron oxide and subjecting such packed castings to the annealing heat, substantially as set forth.

Witness my hand this 8th day of August, 95 1899.

JOHN C. BRADLEY.

Witnesses:

JNO. J. BONNER,  
ELLA R. DEAN.